

Patented Feb. 22, 1927.

1,618,465

## UNITED STATES PATENT OFFICE.

DIRKE NYBAKKER, OF NEW YORK, N. Y.

### FUEL ECONOMIZER.

No Drawing.

Application filed September 23, 1926. Serial No. 137,381.

The composition of matter used for this truly fuel economizer saves about 40% in coal, increases the heat and prevents forming clinkers, soot and ashes and reduces the smoke by its more perfect combustion of the coal.

The invention of this compound was planned with this idea in mind that it should be a genuine saver in fuel and especially in coal so that every user should considerably profit by it.

The improved compound consists of the following ingredients, combined in about the following proportions stated: Powdered saltpeter ten pounds; Glauber salts six pounds; sal ammoniac four pounds; com-

mon salt two pounds; dried sodium sulphate two pounds; powdered borax two pounds; powdered burned umber one pound.

In using the above described powder or composition I dissolve one pound of this compound in ten gallons of water and sprinkle this evenly on the coal when using it, as better results are obtained this way. One ton of coal can be treated with one pound of this compound.

I claim:

A combustion aid for solid fuel comprising a mixture of saltpeter, Glauber salt, sal ammoniac, sodium chloride, borax and burned umber.

DIRKE NYBAKKER.